

## UNITED STATES PATENT OFFICE

2,600,134

DENTAL IMPRESSION COMPOSITION COM-  
PRISING A COPOLYMER OF VINYL CHLO-  
RIDE AND VINYL ACETATE, DI-NORMAL-  
PROPYL PHTHALATE AND A FILLER.Frank J. Sowa, Cranford, and Max M. Schwartz,  
Jersey City, N. J.; said Sowa assignor to said  
Schwartz.No Drawing. Application November 4, 1948,  
Serial No. 58,364.

3 Claims. (Cl. 260—31.8)

1

Our invention relates to compositions for use in taking dental impressions, and is directed particularly to compositions which are characterized by the dimensional stability of the finished impression.

Dental impression compositions developed and used heretofore have in general been of two types; namely, plasters, gums or waxes which set up or harden to form a rigid, stiff or inflexible body; and compositions containing alginates or resins which form relatively softer and more flexible impressions. Plasters, gums and waxes are unsatisfactory because the impression is frequently broken or distorted on being removed from the patient's mouth particularly when teeth are present or there are any undercut or rounded surfaces beneath which the composition extends. Moreover when plaster breaks or crumbles, particles of the plaster may fall into the patient's throat causing serious discomfort or injury. Gums and waxes are further objectionable because they must be introduced into the patient's mouth in a heated condition and often must be cooled by the use of a stream of water or by employing a water-cooled impression tray.

Those compositions which produce a more flexible or resilient impression have the advantage of greater accuracy and ease of removal. However, they have always contained water or volatile solvents which evaporate as the composition sets and after the impression is removed from the mouth. They therefore shrink or become distorted on standing with the result that it is necessary to pour the plaster or stone used in making the model promptly after the impression is taken. Attempts have been made to overcome such dimensional changes by coating the impression with oil or a sealing material but such steps are troublesome, are not always effective, and they frequently cause the loss of detail. The use of solvents is also objectionable because they must be largely evaporated while the composition is in the patient's mouth. Moreover the surfaces of the gums and mouth engaged by the composition are very sensitive and are often tender whereas a great majority of the solvents or liquids usable with gums and resins produce a severe burning sensation when brought into contact with such tissues and therefore cannot be employed in dental impression materials.

Many of the plastic dental impression compounds have other objectionable properties. Thus the alginates will not adhere to most surfaces and therefore require a special perforated impression

2

tray. Moreover, the tray or impression cannot be built up or extended with wax or other materials as is frequently desirable. Other impression compositions are often so stiff that they cause distortion of the surfaces they engage, or they are so flexible and soft that they do not support the plaster or stone used in forming the model so that distortions are introduced during the casting operation.

In accordance with our invention, these objections to compositions of the prior art are overcome and materials are provided for producing dental impressions possessing the desired resiliency and flexibility but having the requisite body to insure the greatest accuracy in the finished impression and resulting models. At the same time, the impressions are characterized by substantially permanent dimensional stability without resorting to the use of sealing materials or coating compounds for preserving the impression. These advantages are preferably attained by employing resinous compounds in combination with a non-volatile plasticizer with or without a solvating agent which converts the resin into a gel-like body under the conditions of use. The resulting impression is found to retain its dimensional stability over long periods of time and does not undergo shrinkage or distortion on long standing.

One of the objects of the present invention is to provide a novel type of composition for use in taking dental impressions.

Another object of the invention is to provide a dental impression composition which is characterized by its flexibility and lasting dimensional stability.

A further object of the present invention is to overcome the objectionable shrinkage and deformation of molding compositions heretofore used in taking dental impressions.

A particular object of the invention is to provide a novel type of impression material embodying a resinous substance and a non-volatile plasticizer with or without a solvating agent.

These and other objects and features of the present invention will appear from the following description thereof in which reference is made to typical compositions and methods of procedure for the purpose of indicating the nature of our invention but without intending to limit our invention thereby.

In general, dental impression materials embodying our invention are produced by mixing a dry powdered resin-containing material with a

liquid plasticizing agent at the time the impression is to be taken. The resin-containing material may include fillers, pigments or other dry ingredients whereas the liquid plasticizer may be mixed with other liquid constituents such as accelerators, buffering agents, flavoring substances or the like.

The preferred type of resinous material used in forming impression compositions for use in dentistry embodies a vinyl resin and particularly copolymers of vinyl chlorideacetate in which the vinyl chloride predominates. The most satisfactory impression composition we have employed are those copolymers containing from 80 to 93% of vinyl chloride, and from 7 to 20% of vinyl acetate. In particular the copolymer containing approximately 90% vinyl chloride and 10% vinyl acetate is used to produce a flexible impression material that has sufficient body to sustain the plaster or stone used in forming a model. When the amount of vinyl chloride in the copolymer is less than 90% the composition is generally softer and more sticky whereas with higher percentages of vinyl chloride in the copolymer it is usually preferable to use an accelerator in order to cause the resin to assume the desired gel-like condition within the time permissible for taking a dental impression.

The resins described may be used in substantially pure state and in finely powdered condition. However, for greater economy, body and smoothness we prefer to employ up to 50% by weight of an inert filler in the powdered product. Typical of such fillers are zinc oxide, talc, powdered limestone or the like. It is usual also to add a pigment, such as cadmium selenide, to the mixture since the imparts the conventional pink color to the impression material. Similarly, a flavoring agent such as oil of peppermint may be added to the dry powder or mixed with the liquid plasticizer to give the composition a pleasing taste.

The plasticizer or solvating agent employed must be chosen so as to be non-toxic and non-irritating to the surfaces engaged by the composition. Moreover, by using those plasticizers which are non-volatile, the dimensional stability of the finished impression is maintained without danger of shrinkage due to evaporation or drying out of the impression on long standing. The number of such plasticizers which may be employed is actually very limited because of the irritation and burning sensation produced by most of the esters commonly used as plasticizers and other compounds which possess plasticizing properties. We have found that the dialiphatic esters of phthalic acid, and particularly those esters in which the total carbon content of the ester group is at least 6, have the necessary plasticizing properties and yet are not irritating to the tender surfaces and tissues they engage. They also blend well with buffering agents such as mineral and vegetable oil and other compounds that might be used as inhibitors.

Dinormal propyl phthalate is the preferred ester to employ since this compound produces substantially no irritation and is an excellent plasticizer for the vinyl chlorideacetate copolymer. However di-allyl phthalate is just as satisfactory as dinormal propyl phthalate and has the same advantages. Di-isopropyl, di-isobutyl, di-n-butyl and dioctyl phthalate are also satisfactory but require an accelerator to set up into the desired final state. Similarly other plastic-

cizing agents may be employed provided they do not produce excessive irritation, are non-toxic, and form a suitable gel. For example, various mixed esters may be employed such as allyl, n-propyl phthalate and ethyl, butyl phthalate. Mixtures of the di-aliphatic esters may be used such as mixtures containing di-allyl phthalate and di-normal propyl phthalate.

By employing accelerators in combination with the plasticizer it is possible to use resinous materials which would otherwise be unsuitable because of the slow action of the plasticizer in converting the resin into a gel-like composition. Similarly plasticizers which have little or relatively slow action on a particular resin may be employed when used in combination with a suitable accelerator. The accelerators, like the plasticizers, must be non-toxic and non-irritating to the tissues. Among the most suitable accelerators that we have used are the esters of aliphatic acids, particularly the esters of acetic acid, although ketones and chlorinated hydrocarbons, ethers and other organic compounds may be employed by themselves or in combination with the esters of aliphatic acids. One of the best accelerators we have used is butyl acetate, but we have also employed ethyl acetate, propyl acetate, isopropyl acetate, amyl acetate and isoamyl acetate. Among the ketones which may be used are diacetone alcohol, di-ethyl ketone, and methyl amyl ketone. Among the ethers which may be used are methyl, ethyl or butyl ethers of ethylene glycol. As chlorinated hydrocarbons we have used carbon tetrachloride and trichlorethylene. The amount of accelerator used varies considerably depending on the type of resin, the type of plasticizer, the type of accelerator and the degree of stiffness or body of the impression desired. Ordinarily the amount of accelerator varies from zero up to about 20% by weight of the liquid used in forming the impression composition. The amount of accelerator may be decreased or eliminated altogether if the liquid used is warmed slightly.

When using accelerators and even when using many of the plasticizers described, it is often desirable to use a diluent or buffering agent such as mineral or vegetable oils. These agents in general have a soothing effect which decreases irritation and permits the use of higher concentrations or different types of the accelerator and plasticizer. The amount of such buffering agent employed may vary from zero to 30% by weight of the liquid used in forming the impression material.

In normal dental practice, it is usually most practical to allow about one minute for the mixing of the liquid with the resin containing powder, one minute for applying the composition to the dental tray and three minutes for the composition to set up into a suitable stable condition in the patient's mouth. When the composition is to set within this time limit, it is usual to employ approximately 25 equal parts by weight of the dry powder resin-containing material to from about 18 to 75 parts of the liquid material. The amount of liquid used may be varied considerably depending on the type of resin and plasticizer used and the consistency of the impression material desired. In a typical case when using 28 grams of resin powder, the amount of liquid plasticizer varies from about 18 to 75 grams.

A preferred composition in which no accelerator or buffering agent is used is as follows:

21 parts by weight of a copolymer of vinyl-chloride-acetate containing 90% vinyl chloride.  
7 parts by weight zinc oxide.

30 parts by weight dinormal propyl phthalate.

If desired from 1 to 5 parts of an accelerator such as butyl acetate may be added to the plasticizer.

The dry materials consisting of the resin and the filler (with any pigment employed) are mixed together in a finely ground or pulverized form. When the impression is to be taken the liquid plasticizer and powder are mixed so as to form a smooth, relatively stiff paste. The paste does not set up at once and may be allowed to stand quite some time without setting, so that the dentist need not rush and may even stop to answer the telephone or attend to other brief duties. Thereafter, the composition may be applied to any conventional impression tray and then inserted into the patient's mouth and pressed into place. As the heat of the human body raises the composition to the temperature of a patient's mouth, the action of the plasticizer is apparently speeded up and the composition is converted into a somewhat stiff, gel-like, elastic body which faithfully conforms to the contours and crevices of the surfaces of the teeth and tissues engaged. Within three minutes after being applied, the impression may be removed and it is then ready to receive the plaster or stone used in forming the model. However it is not necessary to pour the model at once since it may be poured at any time, and even as long as a month or more after after the original impression was taken. Repeated castings may be made from the same impression. Partial dentures made to fit one model will fit another model made from the same impression. It is also found that partial dentures made to fit one model will fit other models made from different impressions of the same mouth. This has never been possible heretofore because of the shrinkage or distortion resulting from evaporation of solvent or dimensional instability of the impression during the casting operation. Moreover, it is not necessary to apply oil or sealing material to the impression in order to preserve it against shrinkage. The steps required in producing and using the impression are therefore simplified whereas the greatest accuracy of the impression is assured.

Instead of using the specific composition referred to above the following composition may be used:

18 parts by weight of vinyl chloride-acetate containing 90% vinyl chloride.  
10 parts by weight of zinc oxide.  
22 parts by weight of di-butyl phthalate.  
2 parts by weight of butyl acetate.

Another alternative composition for the liquid constituents is as follows:

20 parts by weight of ethyl butyl phthalate.  
4 parts by weight of butyl acetate.

A further example of a liquid mixture which may be used is as follows:

20 parts by weight of diallyl phthalate.  
4 parts by weight of mineral oil (Nujol).

Any of the foregoing liquid mixtures may be used with any of the copolymers of vinyl chloride-acetate containing from 80 to 93% of vinyl chloride.

5 The composition may be used for taking impressions for either full or partial dentures or for making crowns, inlays or bridgework. The material is easily removed from the hands, face, dental instruments or the bowl in which 10 it is mixed. It is not capable of reuse and therefore the patient is assured of completely sanitary operation by the dentist.

The dry powdered material and the liquid may be readily packaged and distributed to the 15 dentist and dental technicians and they are immediately ready for use without employing any special equipment. The various alternative compositions which may be produced in accordance with our invention render it possible 20 to supply dentists and dental technicians with impression compositions which are particularly suited to any special needs or technique without departing from the present invention. In view thereof it should be understood that the 25 particular compositions, proportions and methods of employing products embodying our invention as specifically set forth in the foregoing examples are intended to be illustrative only and are not intended to limit the scope of our 30 invention.

We claim:

1. A composition for use in making dental 35 impression material comprising a mixture containing zinc oxide, at least an equal weight of a copolymer of vinyl chloride-acetate and a minor proportion of dinormal propyl phthalate.

2. A composition for use in making dental 40 impressions comprising the product resulting from a reaction between a powder containing a mixture of zinc oxide and at least an equal amount of vinyl chloride-acetate copolymer containing from 80 to 93% of vinyl chloride and a liquid containing from 90 to 95 parts of dinormal propyl phthalate and from 5 to 10 parts 45 of butyl acetate, said liquid and powder being combined in the proportions of approximately 25 parts of powder to from 18 to 75 parts by weight of liquid.

3. A dental impression composition consisting 50 of a gel-like body comprising approximately 25 parts by weight of a copolymer of vinyl chloride-acetate containing from 80 to 93% of vinyl chloride, and from 18 to 75 parts by weight of a solvating agent comprising a major portion 55 of di-normal propyl phthalate and a minor portion of butyl acetate, said composition containing a finely divided inert filler in amount not exceeding the weight of said copolymer.

FRANK J. SOWA.

MAX M. SCHWARTZ.

#### REFERENCES CITED

The following references are of record in the file of this patent:

#### UNITED STATES PATENTS

| Number    | Name      | Date           |
|-----------|-----------|----------------|
| 2,214,127 | Ensminger | Sept. 10, 1940 |
| 2,310,889 | Becker    | Feb. 9, 1943   |
| 2,413,294 | Curtis    | Dec. 31, 1946  |
| 2,428,453 | Field     | Oct. 7, 1947   |
| 2,447,398 | Supinski  | Aug. 17, 1948  |